

1

3,113,054  
QUENCHING OIL AND METHOD OF  
QUENCHING METALS

Michael George Billett and James Gibson, both of Sunbury-on-Thames, England, assignors to The British Petroleum Company Limited, London, England, a British joint-stock corporation  
No Drawing. Filed Mar. 17, 1961, Ser. No. 96,394  
Claims priority, application Great Britain Mar. 18, 1960  
6 Claims. (Cl. 148—29)

Many metal alloys, especially ferrous alloys, require a heat treatment (e.g. at a temperature of 850° C.) followed by rapid cooling to develop the necessary degree of hardness. The hardness of an alloy is mainly dependent upon the formation of a certain physical structure; in the case of steel, the hardness is determined by the proportion of martensite formed during the hardening process. Rapid cooling of the alloy is usually effected by immersing the hot alloy in a relatively cool quenching liquid. A commonly used quenching liquid is mineral oil but for certain alloys, e.g. high-carbon, low-alloy steels straight mineral oils do not form satisfactory quenchants since the initial rate of cooling is too slow. A faster initial cooling rate can be obtained by using water as the quenching medium but this is unsatisfactory for large sections since it cools the metal too quickly at the lower temperatures and often results in distortion and cracking.

We have now developed an improved quenching oil and method of quenching alloys which is particularly suitable in the case of high-carbon, low-alloy steels and other alloys which cannot be satisfactorily cooled in straight mineral oil.

According to the invention there is provided a method of quenching alloys in which there is used a quenching oil consisting of a lubricating oil base containing dissolved therein a small amount of an oil-soluble aluminium compound. (The term oil-soluble is used in the sense that the compound must be capable of remaining in stable suspension in the oil and not separate out of storage. Thus the compound may be present in the oil in the form of a colloidal suspension.)

The lubricating oil is preferably a refined mineral lubricating oil obtained from the distillation of crude petroleum particularly one having a flash point above 350° F. and a Redwood I viscosity at 140° F. not greater than 100 seconds. The viscosity of the quenching oil should also preferably not exceed 100 seconds, e.g. 30–75 seconds, Redwood I at 140° F. If the aluminium compound has a tendency to thicken the lubricating oil, this may be counteracted by the use of an anti-gelling agent e.g. 8-hydroxyquinoline.

The amount of the oil-soluble aluminium compound dissolved in the lubricating oil base is preferably not greater than 10%, e.g. 0.5–5%, by weight of the final composition.

A preferred class of aluminium compounds are the polyoxo-aluminium acylates. These compounds may be prepared by heating aluminium alcoholates with water and carboxylic acids in one or more stages and preferably in an inert, non-volatile diluent such as a light lubricating oil. This method of preparation is described in U.K. patent specification 825,878. Another method of preparation is to heat aluminium alcoholates with carboxylic acids alone so as to liberate alcohol and form acyloxy aluminium alcoholate compounds, and further heat the latter compounds. This method of preparation is described in U.K. patent specification 806,113. Examples of such polyoxo-aluminium acylates are those having the average general formula  $(OAI_{n-1}X)_n$  where  $n$  is an integer greater than 1, preferably 2–10, and  $X$  is an acylate group,

2

i.e. a group having the formula  $RCOO$ — where  $R$  is an aliphatic or aromatic hydrocarbon or substituted hydrocarbon radical, especially a saturated or unsaturated alkyl or aryl radical containing 6–30 carbon atoms. Particularly preferred are such compounds in which the acylate groups are derived from benzoic or salicylic acids, or aliphatic monocarboxylic acids having 12–20 carbon atoms, e.g. stearic or oleic acids. It is to be understood that the acylate groups in any given molecule of the additive may be the same or different and that the additive may consist of a mixture of different molecules.

Another suitable class of oil soluble aluminium compounds are the aluminium glycolates.

The invention also consists in a quenching oil consisting essentially of a lubricating oil having a flash point above 350° F. and a Redwood I viscosity at 140° F. of not more than 100 seconds, e.g. 30–75 seconds, preferably a mineral lubricating oil obtained from the distillation of petroleum, and containing dissolved therein 0.5–5% by weight of the total quenching oil of an oil soluble aluminium compound, particularly one or more of the preferred types of aluminium compound hereinbefore specified, the viscosity of the quenching oil being not greater than 100 seconds Redwood I at 140° F., e.g. 30–75 seconds.

A number of examples of the invention will now be described.

EXAMPLE 1

30 A hardness test was carried out of samples of file steel (a low alloy steel containing 1.23% weight carbon) which had been quenched in a straight mineral lubricating oil and in a quenching oil according to the invention made using the same lubricating oil.

35 The straight mineral lubricating oil (hereinafter called oil L) was obtained from the vacuum distillation of a Middle Eastern crude petroleum oil and had had the normal refining treatment viz dewaxing, solvent refining with furfural, and clay treatment. The refined oil had a Redwood I viscosity at 140° F. of 50 seconds, and a flash point of 400° F.

40 The quenching oil according to the invention (hereinafter called oil Q1) was made by adding 3% by weight of an oil soluble compound M to the above lubricating oil. The aluminium compound M was one commercially available under the trade name "Manalox" and had been prepared as follows:

45 One molecular proportion of aluminium isopropoxide was reacted with two molecular proportions of commercial oleic acid at a temperature increasing to about 220° C. Two molecular proportions of isopropanol distilled off during the reaction a slight vacuum being applied near the end to aid the removal of the last traces of isopropanol. It is believed that the product (M) consisted of a solution in one part by weight of isopropyl oleate of one part by weight of a polyoxo-aluminium acylate of the general formula  $(OAI_{n-1}OCR_1)_n$  where  $R_1$  is an oleyl radical, and  $n$  is 2–10 predominantly 3.

50 Samples of the file steel 0.3" x 1.4" x 4.5" in size were heated for half an hour at 800° C. in an electric furnace and then quenched by plunging them into 5 gallons of the quenchant at room temperature. The quenched samples were then parted slightly off centre on a water cooled slitting wheel giving a transverse section which was ground back to a centre line, polished and then hardness-tested using the well-known Vickers hardness tester. The hardness transverse was made at 0.1" intervals along a line running centrally across the section parallel to its two longer sides. All tests were done in duplicate. The results are given in the following table.

3  
Table

| Distance from short edge of section (inches) | Vickers Hardness Number  |                           |
|----------------------------------------------|--------------------------|---------------------------|
|                                              | Sample Quenched in Oil L | Sample Quenched in Oil Q1 |
| 0                                            | 380                      | 380                       |
| 0.1                                          | 377                      | 378                       |
| 0.2                                          | 368                      | 375                       |
| 0.3                                          | 355                      | 372                       |
| 0.4                                          | 343                      | 370                       |
| 0.5                                          | 335                      | 370                       |
| 0.6                                          | 325                      | 369                       |
| 0.7                                          | 320                      | 369                       |
| 0.8                                          | 325                      | 369                       |
| 0.9                                          | 335                      | 370                       |
| 0.4                                          | 343                      | 370                       |
| 0.3                                          | 355                      | 372                       |
| 0.2                                          | 368                      | 375                       |
| 0.1                                          | 377                      | 378                       |
| 0                                            | 380                      | 380                       |

It will be seen that the use of the quenching oil according to the invention gave a product of much more uniform hardness across its section as compared with the use of the base oil.

## EXAMPLE 2

The initial cooling rate of oils Q1 and L and of an oil (Z) sold commercially as a fast quenching oil, were determined by a nickel ball test. In this test use is made of the well known property of metals in that they lose their magnetism when heated above a certain temperature (the Curie point) which is characteristic for each metal. Nickel was chosen for these quenching tests because of its non-scaling characteristics and resistance to cracking during quenching. The test procedure consisted essentially of heating a nickel ball to 850° C. in a tube furnace then quenching in the oil. The time for the ball to become magnetic gave an accurate measure of the speed of quench from 850° C. to 354° C. (the Curie point of nickel). The results were as follows:

|        | Seconds |
|--------|---------|
| Oil Q1 | 15.5    |
| Oil L  | 22.7    |
| Oil Z  | 19.3    |

It will be seen that from the point of view of fast initial cooling rate, the quenching oil according to the invention was the best of the oils tested.

## EXAMPLE 3

Some chain links of various sizes made from chrome-nickel steel containing 0.4-0.5% weight C, 1.2% weight Ni and 1.8% weight Cr were quenched in the straight mineral lubricating oil L referred to above and in a quenching oil according to the invention (Q2) made by dissolving 5% by weight (based on the final composition) of compound M in lubricating oil L. The quenching system consisted of a continuous conveyor which took the links through a furnace maintained at 850° C. where they remained for approximately 10 minutes before dropping a distance of 1 foot into the quenching bath maintained at 60° C. Rockwell C hardness tests on the treated links showed that in the smaller links (approximately 1/2 inch

long) an increase in surface hardness of 15% was achieved using oil Q2 as compared with when oil L was used. For the larger links (12 inches long, 4 inches wide, 1/2 inch thick) an increase in surface hardness of 10% was achieved. Some of the smaller links were sectioned and an even hardness distribution was found to exist through the section.

## EXAMPLE 4

Some silicon-manganese spring steel stampings (for a refrigerator temperature controller) having a carbon content from 0.6 to 0.7% weight were quenched in the straight mineral lubricating oil L and in the quenching oil according to the invention, Q2. The stampings were passed in an atmosphere of hydrogen through an electrically heated furnace maintained at 900° C. and were discharged into a tank of quenching oil mounted beneath the furnace. The tank contained 40 gallons of oil at a temperature of 60-70° C. When quenching in oil L, a hardness of 530-670 V.P.N. (Vickers pyramid number) was obtained. With oil Q2, hardness values of the order of 750 V.P.N. were obtained, which was similar to that obtained by quenching the steel stampings in water.

We claim:

1. A method of quenching alloys in which there is used a quenching oil consisting of a mineral lubricating oil base containing dissolved therein an oil soluble polyoxo-aluminium acylate compound having the average general formula  $(OAI_2)_n$ , where  $n$  is 2-10 and X is an acylate group of the formula  $RCOO-$  where R is a hydrocarbon radical containing 6-30 carbon atoms, in an amount sufficient to increase the initial rate of cooling of said lubricating oil base.
2. A method according to claim 1, in which the lubricating oil is a refined mineral lubricating oil obtained from the distillation of crude petroleum.
3. A method according to claim 2, in which the lubricating oil has a flash point above 350° F. and a Redwood I viscosity at 140° F. of up to 100 seconds.
4. A method according to claim 1, in which the amount of the oil soluble aluminium compound dissolved in the lubricating oil is 0.5-5% by weight of the quenching oil.
5. A method according to claim 1, in which the acylate groups in the polyoxo-aluminium acylate are derived from at least one of the following acids: benzoic acid, salicylic acid and aliphatic monocarboxylic acids having 12-20 carbon atoms.
6. A method according to claim 1, in which the amount of the oil soluble aluminium compound dissolved in said lubricating oil base is not greater than 10% by weight.

## References Cited in the file of this patent

## UNITED STATES PATENTS

- 2,202,364 Wiezevich ----- May 28, 1940  
 2,744,074 Theobald ----- May 1, 1956  
 2,848,362 Flemmert et al. ----- Aug. 19, 1958  
 2,925,430 Stedehouder et al. ----- Feb. 16, 1960  
 3,054,816 Rinse ----- Sept. 18, 1962

## FOREIGN PATENTS

- 825,878 Great Britain ----- Dec. 23, 1959

UNITED STATES PATENT OFFICE  
CERTIFICATE OF CORRECTION

Patent No. 3,113,054

December 3, 1963

Michael George Billett et al.

It is hereby certified that error appears in the above numbered patent requiring correction and that the said Letters Patent should read as corrected below.

Column 1, line 39, for "separate out of storage" read  
-- separate out on storage --.

Signed and sealed this 28th day of April 1964.

(SEAL)

Attest:

ERNEST W. SWIDER

Attesting Officer

EDWARD J. BRENNER

Commissioner of Patents